

# UNITED STATES PATENT OFFICE.

ALBERT H. EMERY, OF STAMFORD, CONNECTICUT.

## PROCESS OF RAISING THE ELASTIC LIMIT OF METALS AND RELIEVING THEM OF INJURIOUS STRAINS.

No. 894,428.

Specification of Letters Patent.

Patented July 28, 1908.

Application filed November 12, 1907. Serial No. 401,890.

*To all whom it may concern:*

Be it known that I, ALBERT H. EMERY, a citizen of the United States, and resident of Stamford, in the county of Fairfield and State of Connecticut, have invented a certain new and useful Process of Raising the Elastic Limit of Metals and Relieving Them of Injurious Strains, of which the following is a specification.

When metals are loaded with compression, tension or torsion beyond their elastic limit, they take a permanent set and if the strain of compression, tension or torsion is sufficient to make the permanent set very considerable, the elastic limit is raised very considerably. Thus, if a compression member of a bridge is loaded sufficiently to give it a large permanent set of compression, its limit of elasticity will be much raised and the initial strains which were in it before this loading, will be changed, usually much reduced. If a member, such as a bridge link is put under heavy load tension sufficient to give it a large permanent set, the limit of elasticity will be greatly raised and the initial strains which existed in it primarily, will be modified and greatly reduced. If a gun tube is strained by interior strains, such as by introducing into it a heavy hydraulic pressure sufficient to very materially permanently enlarge the tube, the initial strains in this piece will be greatly modified, the limit of elasticity will be greatly raised and when the internal load is removed the metal will take on strains of compression on the interior until these strains balance the remaining strains of tension on the exterior. In like manner, if a coiled spiral spring is loaded with compression sufficiently to give it a very considerable permanent set, its elastic limit will be very materially raised. That is to say, it will, after this overloading, receive a larger loading without permanent set than it would previously and the same is true with a spiral spring if loaded with tension to give it a permanent set. Its limit of elasticity will be raised. Or the load again carried without additional set will be very materially increased. If now very careful tests are made of either the compression column or the tension link or the expanded tube it will be found that the movement caused by added loads giving a curve of pressure, will be different from the movements caused by the removal of those loads. That is to say, if a bar

is under tension its length with increasing loads of fixed amounts successively applied up to its limit of elasticity will be less than the length with the same loads which occur in the gradual removal of these fixed loads. 60 In other words, suppose a load of five parts would load a bar to its limit of elasticity. This bar should stretch one-fifth as much for one part of the load as it does with five; three-fifths as much with three parts as it 65 does with five. It will be found, however, on removing the load, that the bar will be slightly longer with the three parts of the load on, than it was when the load was being put on. It will also be slightly longer when 70 two parts of the load only remain than it was when two parts were put on in the initial loading. Likewise, when we load the spiral spring with compression, if a certain load shows a movement of one inch, the perfect 75 spring would show two inches with twice the load, three inches with three times the load, four inches with four times the load, &c. up to the limit of elasticity; that is to say, the limit from which, when all loads are removed, 80 the spring regains its full length. If now we remove these loads part by part, we will find the spring successively shorter at each point of unloading than it was when it reached the same point in loading. 85

The difference between the lengths of the spring at loading and the corresponding lengths at unloading is what I term the curve of fatigue, and this in the ordinary springs of commerce will often reach with full loads, 90 two, three, four, or even five per cent. of the maximum movement. I desire to get rid of this curve of fatigue, as far as practicable. For this purpose, when the column is compressed or the bridge link extended or the gun tube expanded, or the spring for compression compressed, or the spring which is to be used in tension has been extended, in each case by overloading, I anneal such work after it has been overloaded. This annealing takes out some of the initial strains which are in a piece and enables it to have the loads repeated over and over again with very much less fatigue. That is to say, a spiral spring which has been overloaded by shutting twelve inches and receiving a permanent set of two inches in said shutting will then have an elastic movement of ten inches with this full load. But if we now carefully measure the loads which shut the spring each suc- 100 105 110

cessive inch for the ten inches, and then gradually unload and weigh the load on the spring as the spring reaches each successive inch in opening, it will be found that the loads will be less at each returning inch than were the loads which caused the compression of the spring to the same points. This difference of loading, as I said before, I call the fatigue of the spring. If now I anneal this spring at 5 a proper temperature, which must not be too high, I find that the difference between the curves of loading and unloading will be very greatly reduced. Proper annealing may reduce this difference to one-fourth or one-fifth 10 what it was before the annealing. That is to say, the differences of loading on the return movements after annealing should be not more than one-fourth or one-fifth what they were before the annealing.

20 What I have said applies to columns, links, gun tubes, or springs hardened or unhardened. It has been customary to harden or oiltemper and anneal gun tubes. It has been customary to harden springs. It would be better for the bridges if the compression and tension members were also hardened and annealed. Whether the members mentioned 25 for compression, tension or torsion are hardened or not, they should be treated by the process I have described by overloading in the direction in which the load is applied in the use of such parts and then annealed as described. Such overloading will increase 30 the elastic limit and this annealing after the overloading will remove some injurious strains and will greatly reduce the curve of fatigue. This is also true of parts which are hardened very much and then annealed to temper them when they may be much over- 35 loaded in the direction of use, receiving a large permanent set and a great increase of elasticity and then again annealed. This annealing after the straining will in general be at a lower heat than should be the annealing 40 to temper them after they are hardened.

45 This over-straining the parts to raise the limit of elasticity and then annealing to remove injurious strains may be done once or twice and sometimes thrice with profit, each 50 time the limit of elasticity being raised higher and the part being enabled to carry a higher load without injury, or the overloading may be repeated, followed by a single annealing.

55 In the case of a spring that has not been made very hard when hardening, it may receive its overload without annealing for temper, and permanent set given it before annealing at all, and then, after annealing, it 60 may, if desired, again be overloaded and re-annealed at a somewhat lower temperature. But the best springs would be made over-hard at the outset, then annealed for temper before loading, then overloaded to give a 65 large permanent set by a load once or twice

repeated and then annealed at a somewhat lower temperature than the first annealing, and this process of overloading and again annealing may be repeated one or more times if desired.

I have mentioned this process as being applied to separate pieces, but it may be used with several parts in combination in the same way in principle and plan as shown applied to single pieces and when properly applied to structures, the different members of the structure will be better able to perform their functions properly.

In all cases, the annealing of strained parts which have not been hardened before straining, should be at a temperature not sufficient to reduce the apparent limit of elasticity below what it was before straining, nor should it be sufficient to much reduce the limit of elasticity from that point to which it has been raised by the overloading. And in case of those parts which have been hardened previously to straining, the annealing after heavy final straining should be at a temperature not sufficient to reduce the limit of elasticity much if any below that which the part had before overloading or straining. And in general, this final annealing after straining, should be at a temperature lower than that at which the piece should be annealed when it requires softening before straining.

Having thus described my invention, what I claim and desire to secure by Letters Patent is:—

1. The process of treating metals, for the purpose of raising their elastic limit and relieving them from injurious strains, which consists in loading a part made from the metal, in the direction of the load which it is to bear when in use, sufficiently to give it a permanent set and increase its limit of elasticity and then annealing it at a low temperature not sufficient to much reduce the limit of elasticity, but sufficient to reduce the curve of fatigue.

2. The process of treating metals, for the purpose of raising their elastic limit and relieving them from injurious strains, which consists in repeatedly loading the metal in the direction of the load which it is to bear when in use, sufficiently to give it a permanent set and increase its limit of elasticity and then annealing it at a low temperature not sufficient to much reduce the limit of elasticity, but sufficient to reduce the curve of fatigue.

3. The process of treating metals, for the purpose of raising their elastic limit and relieving them from injurious strains, which consists in repeatedly loading the metal in the direction of the load which it is to bear when in use sufficiently to give it a permanent set and increase its limit of elasticity and then annealing it at a low temperature not sufficient to reduce the limit of elasticity,

but sufficient to much reduce the curve of fatigue, then repeating said steps of loading and annealing in the order named.

4. The process of treating metals for the purpose of raising their elastic limit and relieving them from injurious strains, which consists in first hardening the metal, then loading it in the direction of the load which it is to bear when in use sufficiently to give it 10 a permanent set and then annealing it, substantially as set forth.

5. The process of treating metals for the purpose of raising their elastic limit and relieving them from injurious strains which

consists in first hardening the metal, then 15 tempering it by annealing, then loading it in the direction of the load which it is to bear when in use, sufficiently to give it a permanent set, and then annealing it substantially as set forth.

The foregoing specification signed at Washington, D. C., this 12th day of November, 1907.

ALBERT H. EMERY.

In presence of—

HERVEY S. KNIGHT,  
EDWIN S. CLARKSON.